

# UNITED STATES PATENT OFFICE.

JAMES G. B. PERKINS AND JULIUS B. B. STRYKER, OF LANSDALE, PENNSYLVANIA,  
ASSIGNORS TO PERKINS GLUE COMPANY, A CORPORATION OF PENNSYLVANIA.

## PROCESS OF MAKING VEGETABLE GLUE.

1,378,128.

Specification of Letters Patent. Patented May 17, 1921.

No Drawing.

Application filed September 26, 1917. Serial No. 193,240.

To all whom it may concern:

Be it known that we, JAMES G. B. PERKINS and JULIUS B. B. STRYKER, citizens of the United States, and residents of Lansdale, 5 in the county of Montgomery and State of Pennsylvania, have invented certain new and useful Improvements in Processes of Making Vegetable Glue, of which the following is a specification.

10 Our invention relates to improvements in processes of making vegetable glue. More particularly, the invention relates to processes of making a substantially neutral vegetable glue having substantially the 15 qualities of animal glue for gluing up veneers and the like.

In U. S. Reissue Letters Patent No. 13436, dated July 2, 1913, and in U. S. Letters Patent Nos. 1,020,656, 1,078,691, 1,078,692 and 20 1,200,488, there are disclosed methods of making vegetable glue by dissolving a starchy carbohydrate with caustic alkali, such as caustic soda, the resulting glue being markedly alkaline. Even if the percentage 25 of caustic alkali be reduced to about 3%, based on the dry weight of the starch and heat be used to aid the solution of the starch, the resulting glue is sufficiently alkaline so that when applied to very thin veneers, it 30 will cause a discoloration of the wood veneer, which discoloration may appear on the opposite side of the wood layer from that on which the glue is applied. In many cases this discoloration is not a serious 35 disadvantage, and with the thicker veneers it is not objectionable or does not appear at all. With certain kinds of wood and in certain cases, especially where very thin layers of wood are being glued together, this discoloration or staining may be a detriment, 40 which it is desirable to avoid.

The main object of the present invention is to provide a vegetable glue having substantially the properties of the glue described in 45 said U. S. Letters Patent, but which is so made or treated that this discoloration or staining is avoided. It is also desirable to provide a vegetable glue for this purpose which is somewhat more fluid than that 50 hitherto in use. Further objects, features and advantages will more clearly appear from detailed description given below.

In producing the new glue, we take a suitable starchy carbohydrate, preferably the 55 glue base resulting from the preliminary

treatment described in either of said U. S. Letters Patent. However, certain starches appear on the market which require no preliminary treatment, and these may be used, if desired. Whether such starch is suitable 60 may be easily determined by testing the same. We preferably use cassava starch or tapioca flour.

To make the glue, a suitable starchy carbohydrate is preferably dissolved with about 65 3 parts or less by weight of water and about 3% by weight of caustic soda, the caustic soda being added in the form of a 33% solution. The starch is first thoroughly mixed with the water and then the caustic soda 70 solution added gradually with continual stirring, until the batch is transformed from a mixture of suspended starch in water to a homogeneous colloidal solution of starch, alkali and water, having substantially the 75 properties of good animal glue for gluing up high grade wood veneers, as described in said Letters Patent. The resulting glue, although thick and viscous, is capable of flowing through pipes 2 inches in diameter, is 80 capable of being spread by glue applying machinery and has substantially the adhesive qualities of animal glue for this class of work.

To prevent this glue from discoloring and 85 staining the wood, as above described, we add thereto a neutralizing agent after the alkali has acted upon the starch so as to make the glue substantially neutral. While 90 various neutralizing agents have been suggested, we have found that certain ammonia salts have distinct advantages over certain other neutralizing agents, and we prefer ammonium sulfate or ammonium chlorid. In selecting the neutralizing agent and applying the same, we believe it to be important 95 to avoid conditions of electrolytic dissociation or changed concentration tending to flocculate the colloid glue. While it is probably true that, not only is the ammonium chlorid or sulfate itself an electrolyte, but also the sodium chlorid, or sulfate, formed with the caustic soda already in the glue is an electrolyte, nevertheless, we believe that the ammonium ion, by reason of 100 its temporary presence in the solution, decreases the degree of dissociation and therefore decreases the flocculating action of the sodium salts produced, and by reason of its gradual, progressive and partial elimina- 105 110

tion, serves to avoid the sudden change of electrostatic condition in the colloidal mass that might result in flocculating the starchy carbohydrate. While we believe that the 5 ammonia is largely if gradually eliminated from the glue, a certain amount of it seems to linger in the glue for a considerable time as free alkali, which we believe has the action of preventing flocculation of the glue 10 above referred to, but which does not act to cause staining or discoloration of the wood. For the purposes of the invention, therefore, the glue is substantially neutral in the sense of not staining the wood. We prefer to add 15 the ammonium salt to the glue in the form of a fine powder in sufficient quantity to substantially neutralize the glue in that the caustic alkali is substantially neutralized. However, these ammonia salts may be added 20 in the form of a solution. In either case, it is preferable to add the neutralizing agent while the glue is still hot or warm and indeed, we prefer to apply the glue to the wood or other articles being joined while 25 it is still warm, especially if made up with about 3% or less of caustic soda. The amount of neutralizing agent required may be easily calculated from the amount of alkali used in making the starch glue solution. 30 While these ammonia salts are substantially neutral they act in a sense like an acid in neutralizing the caustic alkali in the glue, combining with the caustic to produce non-caustic salts or bases which are eliminated from the liquid phase by reason of 35 their being volatile or being inert precipitates.

The neutralizing agent should be thoroughly stirred in so that it is brought into 40 intimate mixture with all parts of the glue. We also find it advantageous to add with the dry powder neutralizing agent about an equal weight of silicious material, such as, finely ground feldspar, quartz or silica. In 45 stead of caustic soda for dissolving the starch, other alkaline compounds may be used. Preferably, less than 12% by weight of caustic alkali is used in dissolving the starch.

50 While we prefer to heat the mixture during the dissolving of the starch, the temperature being carefully kept considerably below 175° F., yet if more than 3% of caustic alkali is used, as, for example, 8%, the 55 solution of the starch may be brought about without heating the batch. By carefully regulating the heat, even less than 3% of caustic alkali may be used. If heat is used, it should be carefully regulated to prevent 60 local overcooking of the starch, or overcooking by long continued relatively high temperature, as described in Perkins' application, Serial No. 808739, filed Dec. 26, 1913, now Patent No. 1,251,275 issued Dec. 25, 65 1917.

If, on standing a considerable time, the glue thickens up, so that it is too viscous and does not flow readily enough, it may in most cases be brought back to proper condition by heating it up to 130-140° F. and thoroughly 70 stirring it.

While the amount of water used in the process may be varied somewhat, we preferably use  $2\frac{1}{8}$  to  $2\frac{1}{4}$  parts of water by weight, based on the dry starch base used. The neutral neutralizing agent when added should be thoroughly stirred in, so that all parts of the batch will have an opportunity to be acted upon thereby. The addition of the silicious filler seems to increase the adhesive 80 strength of the glue, or prevent the adhesive strength of the glue from being materially decreased. It is, of course, not necessary that the neutral glue be used for joining layers of wood, as it may be found advantageous for joining fabric to wood and for joining other articles, but by the method described the glue is rendered substantially neutral without materially decreasing its strength or spreadability or materially affecting its essential properties for furniture veneering and the like. 85

While we have described our improvements in great detail and have given certain examples, we do not desire to be limited thereto, since many changes may be made and other reagents used, as will be understood by those skilled in the art. It is desired to cover all the modifications coming 90 within the language of the appended claims. 100

What we claim as new and desire to secure by Letters Patent is:

1. The process of making vegetable glue which consists in dissolving a starchy carbohydrate in caustic alkali and about 3 105 parts or less by weight of water and heat below 175° F., the carbohydrate being such that the resulting alkaline solution has substantially the properties of animal glue for gluing up high grade veneers and substantially neutralizing the glue with an ammonia salt without materially decreasing its 110 strength or spreadability.

2. The process of making vegetable glue which consists in dissolving a starchy carbohydrate with caustic alkali and about 3 115 parts or less by weight of water and heat below 175° F., the carbohydrate being such that the resulting alkaline solution has substantially the properties of animal glue for 120 gluing up high grade veneers, and then substantially neutralizing the glue with ammonium chloride without materially decreasing its strength or spreadability.

3. The process of making vegetable glue 125 which consists in dissolving a starchy carbohydrate with caustic alkali and about 3 parts or less by weight of water and heat below 175° F., the carbohydrate being such that the resulting alkaline solution has sub- 130

stantially the properties of animal glue for gluing up high grade veneers, and then adding an ammonia salt while still warm to substantially neutralize the glue.

- 5 4. The process of making vegetable glue which consists in dissolving a starchy carbohydrate with caustic alkali and about 3 parts or less by weight of water and heat below 175° F., the carbohydrate being such 70 that the resulting alkaline solution has substantially the properties of animal glue for gluing up high grade veneers, and adding a salt of ammonia in dry powdered form to substantially neutralize the glue without 75 materially decreasing its strength or spreadability.

- 10 5. The process of making vegetable glue which consists in dissolving a starchy carbohydrate with caustic alkali and about 3 parts or less by weight of water and heat 80 below 175° F., the carbohydrate being such that the resulting alkaline solution has substantially the properties of animal glue for gluing up high grade veneers, and then adding 85 an ammonia salt to substantially neutralize the glue, and a silicious filler.

- 15 6. The process of making vegetable glue which consists in dissolving a starchy carbohydrate with caustic alkali and water, the carbohydrate being such that the resulting alkaline solution has substantially the properties of animal glue for gluing up high grade veneers, and substantially neutralizing the glue with an ammonia salt 90 without materially decreasing its strength or spreadability.

- 20 7. The process of making vegetable glue which consists in dissolving a starchy carbohydrate with water and an alkaline compound 95 pound, the carbohydrate being such that the resulting solution is a thick viscous alkaline mass capable of flowing through pipes two inches in diameter, and of being spread by glue applying machinery and of adhesively securing layers of wood together, and adding 100 an ammonia salt thereto to substantially neutralize the glue without materially decreasing its strength or spreadability.

- 25 8. The process of making vegetable glue which consists in dissolving a starchy carbohydrate with about 3 parts or less by weight 105 of water and an alkaline compound, the carbohydrate being such that the resulting solution is a thick viscous alkaline mass capable of flowing through pipes two inches in diameter, and of being spread by glue applying machinery and of adhesively securing layers of wood together, and adding an ammonia salt thereto to substantially neutralize the glue without materially decreasing 110 its strength or spreadability.

- 30 9. The process of making vegetable glue which consists in dissolving a starchy carbohydrate with caustic alkali and water, the carbohydrate and proportions being such 115

that the resulting alkaline glue solution has substantially the properties of animal glue for gluing up veneers, and substantially neutralizing the glue with a substantially neutral salt without materially decreasing its 70 strength or spreadability, said salt combining with the caustic to produce a non-caustic salt or base which is eliminated from the liquid phase by reason of its being volatile or an inert precipitate. 75

10. The process of making vegetable glue which consists in dissolving a starchy carbohydrate base with water and an alkaline compound, the carbohydrate and proportions being such that the resulting alkaline 80 glue solution has substantially the adhesive properties of animal glue for gluing up high-grade wood veneers and is viscous but capable of being spread by glue-applying machinery, and substantially neutralizing 85 the glue with a substantially neutral material without materially decreasing its strength or spreadability, said neutral material combining with the alkaline compound to produce a non-caustic salt or base which is 90 eliminated from the liquid phase by reason of its being volatile or an inert precipitate.

11. The process of making vegetable glue which consists in dissolving a starchy carbohydrate base with an alkaline compound 95 and about 3 parts or less by weight of water, the carbohydrate being such that the resulting alkaline glue has substantially the adhesive properties of animal glue for gluing up wood veneers and is viscous but capable of flowing through pipes two inches in diameter and of being spread by glue-applying machinery, and substantially neutralizing the glue with a substantially neutral compound without materially decreasing its 100 strength or spreadability, said compound combining with the alkaline compound to produce a non-caustic salt or base which is 105 eliminated from the liquid phase by reason of its being volatile or an inert precipitate. 110

12. The process of making vegetable glue which consists in dissolving starch with caustic alkali in about 3 parts or less by weight of water, the condition of the starch being such that the resulting alkaline glue 115 solution has substantially the properties of animal glue for gluing up veneers, and substantially neutralizing the glue with a salt which combines with the caustic to produce therewith non-caustic products without materially decreasing the strength or spreadability of the glue.

Signed at Lansdale in the county of Montgomery and State of Pennsylvania this 22nd day of September, A. D. 1917.

JAMES G. B. PERKINS.

JULIUS B. B. STRYKER.

Witnesses:

EARLY L. GILBERT,  
I. E. MOORE.